

J. A. POTTER.  
APPARATUS FOR SMELTING ORES.  
APPLICATION FILED DEC. 23, 1912.

1,113,481.

Patented Oct. 13, 1914.

3 SHEETS-SHEET 1.

FIG. 1



WITNESSES

H. B. Keating  
Leon Boillet

INVENTOR

John A. Potter  
By Francis M. Wright  
his attorney

J. A. POTTER.  
APPARATUS FOR SMELTING ORES.  
APPLICATION FILED DEC. 23, 1912.

1,113,481.

Patented Oct. 13, 1914.

3 SHEETS—SHEET 2.



**WITNESSES**

N. B. Keating  
Dear Brother

INVENTOR  
John C. Potter  
By  
Francis M. Wright  
his attorney

1,113,481.

J. A. POTTER.  
APPARATUS FOR SMELTING ORES.  
APPLICATION FILED DEO. 23, 1912.

Patented Oct. 13, 1914.

3 SHEETS-SHEET 3.

FIG. 4.



FIG. 3



WITNESSES

N. B. Keating  
Leon Boillot

INVENTOR

John A. Potter  
Francis L. Wright  
his ATTORNEY

BY

# UNITED STATES PATENT OFFICE.

JOHN A. POTTER, OF PUEBLO, COLORADO.

## APPARATUS FOR SMELTING ORES.

1,113,481.

Specification of Letters Patent. Patented Oct. 13, 1914.

Application filed December 23, 1912. Serial No. 738,245.

To all whom it may concern:

Be it known that I, JOHN A. POTTER, a citizen of the United States, residing at Pueblo, in the county of Pueblo and State 5 of Colorado, have invented new and useful Improvements in Apparatus for Smelting Ores, of which the following is a specification.

The object of the present invention is to 10 provide an improved apparatus for separating metals such as gold, silver, iron, copper, lead, zinc, antimony and bismuth from ores, drosses, mixtures, mattes, slags, and the like.

In the accompanying drawing, Figure 1 15 is a plan view of my improved apparatus, certain parts being broken away; Fig. 2 is a broken longitudinal vertical section on the line 2—2 of Fig. 1; Fig. 3 is a vertical cross section on the line 3—3 of Fig. 1; Fig. 4 is a vertical cross section on the line 4—4 of Fig. 2.

Referring to the drawings, 1 indicates concrete foundations, on which are supported 20 steel columns 2, and fire brick walls 3, strengthened and bound together by plates 4 and brace staves 5, which bind together the walls of the gas-producing chamber 6 and fusion chamber 7.

8 indicates an ore shaft, and 9, 9' condensing regenerating flues, the rear ends of 25 which communicate with an air supply pipe 12 controlled by a valve 10, and leading upwardly from a blast pipe 24 and also communicating with an upwardly leading exhaust pipe 12', said communications being controlled by a butterfly valve 11.

13 indicates an inclined plate located at 30 the bottom of the ore shaft 8, on which plate is made to move a ram 14 and on 40 which plate are secured shaft bearings 15 and 15', in which bearings is a shaft 16 having secured thereon a sprocket wheel 21 and cams 17 and 17', that revolve inside eccentricities 18 and 18', connecting with lugs 19 and 45 19' of the ram 14 by a shaft 20.

Connected to the lower end of the gas-producing chamber 6 is a pipe 22 controlled by a valve 23 and leading from the blast pipe 24. An oil or gas pipe 25 connects 50 with the chamber 6 above the air pipe 22, and in the upper portion of the rear wall in said chamber 6 is an opening 26' covered by a door 26. At the bottom of the sides of the chamber 6 are clearing doors 45, 45'.

55 The condensing and regenerating flues 9

and 9' open into the fusion chamber 7 by ports 27 and 27'. The regenerating flues contain a longitudinal series of baffling walls 28, 28', and in the lower portions of said flues are a series of basins 29, 29' having spouts 30 and tap holes 30'.

31, 31' indicate ladles suspended by harness from carriages 32, 32' running on rails 33, 33'.

34 indicates an ore-charging car, running 65 on rails 35, 35'.

36 indicates a furnace door, 37 a slag and metal spout and 38, 38' inwardly flaring holes for the insertion of a bar through the furnace wall.

39 and 39' indicate oil or gas pipes, 40 and 40' platforms, and 41, a furnace door lever.

42 indicates the ore mixture embankment, 70 43 a sheave wheel on the butterfly valve 11, and 44 a hand rope over wheel; while 46 75 indicates the twyer holes connecting the chambers 6 and 7.

47 indicates the liquid metal, 48 the slag tap hole and 48' the metal tap hole below the slag hole 48, 49 the settling ladle, and 80 50 the slag floating on the liquid matte or metal in the chamber 7.

The ores or materials to be treated may 85 contain one or more metals, or carbonates or oxids of metals in combinations comprising gold, silver, iron, copper, lead, zinc, antimony, bismuth and the like. As an example, we will suppose that the material to be treated contains oxid of iron, copper, lead and zinc with a small percentage of sulfur,

which ores are crushed and mixed with fluxes, to about corn size or smaller. These are fed into the shaft 8, and fall on to the plate 13.

The charging operation is continued until the stack 8 is full, at which 90 time a portion of the charge has passed forward over the twyer holes 46 into the melting chamber 7, there forming the embankment of ore mixture 42.

Now, at this time, fire is started in the chambers 7 and 6 by 95 first admitting air under pressure through the valve 10 and butterfly valve 11 into and through the condensing and regenerator flue 9, down through the port 27, where oil or

gas, flowing from the pipe 39, is encountered, and where ignition, combustion, and heated gas are produced, which fills the chamber 7, and passes therethrough around the face of the ore 42, into and up the port 27', into and through the condensing and 100 105 110

regenerating flue 9', into and through the butterfly valve 11, into the pipe 12, whence it is conveyed for further treatment. Now after about one hour's time the course of air, fuel and gas currents are reversed, by pulling down on the hand rope 44, causing the wheel 43 and butterfly valve 11 to rotate about one-fourth of a revolution, thus causing the air blast to pass into and through the condensing flue 9', down and into the port 27' where it encounters oil or gas which instead of flowing through the pipe 39 has been caused to flow through the pipe 39', where ignition and combustion, now take place and the resulting gas travels through the chamber 7 through the port 27, and into and through the condensing and regenerating flue 9, into and through the valve 11 and pipe 12, as before stated, for further treatment. Now while these reversals are proceeding intermittently, fire is also started in the gas-producing chamber 6, by admitting into said chamber air through the valve 23, when it encounters oil or gas flowing through the pipe 25, whereupon ignition and combustion are produced, the resulting gases passing through the twyer holes 46 into and through the ore 42 and into the chamber 7, there associating and moving with the heretofore described gas currents passing through said chamber 7.

Now after all the parts have reached the proper heat conditions for operations, the temperatures and the characters of the gases produced are regulated by adjusting the air and fuel supply so as to produce and maintain a hot reducing gas in chamber 6 of about 2000° F. which gas at such a temperature and under sufficient pressure permeates and commingles with the crushed ore mixture 42, there combusting the oxygen associated with the ore mixture, thereby forming metallic particles of zinc, lead, copper, iron, and matte. The zinc particles when formed immediately become volatilized and pass into chamber 7 with the reducing gas currents, while the iron, copper, lead and the like form matte particles that begin to liquefy and precipitate to the bottom of the chamber 7, and accumulate at the point 47, under the liquid slag formed by the fusion of earths, fluxes, and the like. Now while these actions are proceeding, fluid fuel and air are supplied in such proportions by the conduit 39 or 39', and flue 9 or 9' that highly heated reducing gas is being produced under sufficient pressure at port 27 or 27', as the case may be, that penetrates, fuses and liquefies the exposed faces of the de-oxidized ore embankment 42, forming thereon a liquid slag blanket, that fuses from the ore faces on to the chamber bottom, while setting free the particles of lead, copper, or iron matte, that in turn liquefy and pre-

cipitate on to the furnace hearth under the liquid slag according to their specific gravity, while the fusing hot gas also associates with the reducing gas containing the zinc vapor issuing from the ore faces, thus protecting them from oxidation, and the combining gas currents then pass out of the chamber 7 under pressure into and through port 27' or 27, up into condensing flue 9' or 9, where they encounter baffling walls 28' or 28, and there give up the zinc vapor, which condenses, falls and accumulates in a liquid state in the basins 29' or 29. Finally the cooled, shrunk, monoxid gas passes through the valve 11 into the pipe 12, whence it is conveyed for further treatment and uses, as it still contains metallic and calorific values.

Now as the above outlined actions are proceeding, the ore embankment is being renewed as fast as its faces are fused away, since the ram 14 is caused to move forward and backward on the plate 13 by mechanical power applied to the wheel 21, shaft 16, cams 17 and 17', eccentrics 18 and 18', shaft 20, to lugs 19 and 19', of the ram 14, thus causing the descending ore mixtures to be crowded forward over the twyer holes 46 into the chamber 7, while at the same time new ore mixtures are being fed into the top of the ore shaft 8.

While the above operations are proceeding, the newly formed unvaporized metals and mattes are being liquated and precipitated; the lead to the bottom of the chamber, while the copper floats on the lead, and the matte in turn floats on the copper, and the slags float on the matte at the point 47, whence they are withdrawn at intervals through the tap holes 48 and 48' and spout 37 into the ladle 49 and thence removed as desired. In the meantime, the condensed zinc vapors have been accumulating in the basins 29 or 29', from which they are withdrawn alternately, just prior to the reversals of the air, fuel and gas currents. Hence it will be seen that a continuous process is obtained.

Should it be desired to extract volatilizable metal or metals from metallic mixtures, ores, and the like by volatilization and condensation only, and not to fuse to a liquid the ore mixture, operations are carried on the same as above with certain exceptions. Less heat is maintained in the chamber 7, thereby sintering the ore mixture only, thus necessitating its removal from the chamber 7 by hand rakes through the door 36, during which time all heat operations cease and about two-thirds of the ore embankment is withdrawn, after which the door 36 is closed and operations resumed.

Carbon or hydrocarbons may be mixed with ore mixture as coal, coke, peat, wood, asphaltum, and the like, in finely divided state, which mixture is gasified by the heat

70

75

80

85

90

95

100

105

110

115

120

125

130

obtained from the combustion of fuel and air in the chamber 7, while the gases generated from the charring mixture of hydrocarbons and ore consume the oxygen in the ore mixture, reduce the metals, and volatilize, carry and protect them from oxidation, while they associate themselves with the gases passing through the chamber 7 as before explained. In this case, the deoxidized ore mixture can be converted into a slag, setting free any non-volatilizable metals as before outlined, or it can be withdrawn from the chamber 7 in a sintered state, and it should be understood that, while the gasifying action is proceeding, air can be admitted into the chamber 6, then into and through twyer slot 46, into contact with the ore and carbonaceous mixture, thereby causing rapid combustion and gasification. Oxidation of the volatilized metals can be produced by this arrangement when extracting either one or more metals in which case the operations and constructions are slightly modified. First, instead of a reducing gas being maintained in the chamber 7, an oxidizing atmosphere is produced, thereby oxidizing the metal vapors and gas issuing from the faces of ore embankment 42, thus forming an oxid dust or powder of the volatilized metals, that, with the burnt gas, travels through and out of the chamber 7 into the ports 27 and 27', into the regenerating fives 9 or 9', from which the baffling walls may have been removed to give free passage to the cooling gases and oxid dusts, which finally pass into the pipe 12 and are then conveyed to a filtering department, as a bag house, or the like, where the oxid dusts are obtained.

It is understood that the above process is conducted either continually or intermittently, as when melting the ore mixture into a liquid, or where it is withdrawn from furnace in a sintered state, and that a carbon or hydrocarbonaceous mixture or reducing gas can be utilized for deoxidizing agents in the ore embankment 42. When employing this arrangement for reducing oxid of iron to wrought or cast iron from ores containing iron alone, or associated with one or more volatilizing metals, the process is carried on about as in the first case, with the following differences. When making wrought iron, the ore is mixed with fluxes and limited amounts of carbonaceous materials charged and deoxidized with gas from the chamber 6. At the same time a highly heated reducing atmosphere is maintained under a suitable pressure in chambers 6 and 7, when the fluxes and earths from slag that become liquid and liqueate from face of the ore embankment 42 on to the furnace hearth 50, leaving the reduced wrought iron particles on the face of ore embankment, which in a short time form a crust of wrought iron of honey-comb

formation. When this crust becomes about 2 inches thick the gas pressure and currents are reduced in chambers 6 and 7, and workmen insert hooked bars into and through the holes 38 and 38' into the chamber 7 and proceed to peel off the crust of wrought iron from the ore embankment and form same into balls by pressing it against the side walls of the furnace, thus welding the metal together into balls of about 20 inches in diameter, which are then withdrawn from the chamber 7 through the door 36 and further treated as desired. Now this peeling and balling is intermittent, and requires about 20 minutes for each peeling, balling and extracting, after which time the process is renewed, and a new crust is formed in about 30 minutes' time, while feeding the ore and tapping slag is proceeding. Should the ore mixtures contain volatilizable metals, they pass off with the gas into condensing flue 9 or 9', and are recovered, as before explained.

To produce cast iron the process is carried on similarly to that when making wrought iron, except that excess carbon or hydro-carbonaceous materials are mixed with the ores, and air, cold or pre-heated, is blown into the chamber 6, then through the twyer slot 46, there permeating and combusting the fuel mixture in ore embankment; thus deoxidizing the ore, also carbonizing the recovered metals while melting, which then precipitate on to the hearth under the slag which is then forming, whence they are intermittently withdrawn and dispensed with as desired. I have employed this method to convert steel and wrought iron clippings, borings, turnings and the like into cast iron, by mixing carbonaceous materials with the metals and melting the mixture with flame from the port 27 or 27', thus melting the faces of embankment away and bringing the metal particles into close contact with the incandescent carbon and the reducing gases, whereby carbon is then absorbed. I may add that, by this same treatment, cast iron, as pig, scrap, borings, turnings, and the like, have been successfully melted and their metaloids, as carbon, silicon, manganese, and the like, preserved while melting, thus opening up a new field in general foundry work, as melting by oil or gas is cheaper and quicker than with coke.

Coal can be gasified in the chamber 6 and a coal fired furnace could be used to furnish a fusing flame, and a stack can be added, but I find that to combust the fuel, an under sufficient pressure is far more effective and economical, as then the reducing gas maintained in the ore body and chambers 6 and 7 and regenerator flues promote better conditions to deoxidize, volatilize, and protect the metals from oxi-

dation, as all outside air is excluded by the internal pressure, while a stack draft causes oxidation by the air passing into the chamber 7 and flues 9 and 9' through the 5 numerous crevices and cracks in the furnace walls, which result would render the process much less useful and effective.

I claim:—

1. In an apparatus of the character described, the combination of a furnace having a rear wall, through a central opening in which ore to be treated is charged, condensing and regenerating flues opening through said rear wall on opposite sides of said central charging opening, an exhaust conduit, a pipe for conducting air under pressure, means for connecting either of said flues with said pipe, and the other with said exhaust conduit, and means in said flues for condensing metallic vapors, and for separating from said flues the liquefied metal resulting from the condensation of said vapor.
2. In an apparatus of the character described, the combination of a furnace having a rear wall, through a central opening in which ore to be treated is charged, condensing and regenerating flues opening through said rear wall on opposite sides of said central charging opening, conduits for fluid 30 fuel discharging adjacent to the openings of said flues into said furnace, an exhaust conduit, a pipe for conducting air under pressure, means for connecting either of said flues with said pipe, and the other with said 35 exhaust conduit, and means in said flues for condensing metallic vapors, and for separating from said flues the liquefied metal resulting from the condensation of said vapor.
3. In an apparatus of the character described, the combination of a furnace having a rear wall, through a central opening in which ore to be treated is charged, said rear wall being formed immediately beneath said charging opening with a small opening for 40 permitting the passage of a gas to said furnace through the body of ore charged thereto from said charging opening, an exhaust conduit, a pipe for conducting air under pressure, means for connecting either of said flues with said pipe, and the other with said 45 exhaust conduit, and means in said flues for condensing metallic vapors, and for separating from said flues the liquefied metal resulting from the condensation of said vapor.
4. In an apparatus of the character described, the combination of a furnace having a rear wall, through a central opening in which ore to be treated is charged, said rear wall being formed immediately beneath said charging opening with a small opening for 50 permitting the passage of a gas to said furnace through the body of ore charged thereto from said charging opening, and said apparatus having a gas producer chamber connected with said small opening, an exhaust conduit, a pipe for conducting air under pressure, means for connecting either of said flues with said pipe, and the other with said exhaust conduit, and means in said flues for condensing metallic vapors and 55 for separating from said flues the liquefied metal resulting from the condensation of said vapor.
5. In an apparatus of the character described, the combination of a furnace having a rear wall, through a central opening in which ore to be treated is charged, said rear wall being formed immediately beneath said charging opening with a small opening for 60 permitting the passage of a gas to said furnace through the body of ore charged thereto from said charging opening, and said apparatus having a gas producer chamber connected with said small opening, an exhaust conduit, a pipe for conducting air under pressure, means for connecting either of said flues with said pipe, and the other with said exhaust conduit, and means in said flues for condensing metallic vapors and 65 for separating from said flues the liquefied metal resulting from the condensation of said vapor.
6. In an apparatus of the character described, the combination of a furnace having a rear wall, through a central opening in which ore to be treated is charged, said rear wall being formed immediately beneath said charging opening with a small opening for 70 permitting the passage of a gas to said furnace through the body of ore charged thereto from said charging opening, and said apparatus having a gas producer chamber connected with said small opening, an exhaust conduit, a pipe for conducting air under pressure, means for connecting either of said flues with said pipe, and the other with said exhaust conduit, and means in said flues for condensing metallic vapors and 75 for separating from said flues the liquefied metal resulting from the condensation of said vapor.
7. In an apparatus of the character described, the combination of a furnace having a rear wall, through a central opening in which ore to be treated is charged, said rear wall being formed immediately beneath said charging opening with a small opening for 80 permitting the passage of a gas to said furnace through the body of ore charged thereto from said charging opening, and said apparatus having a gas producer chamber connected with said small opening, means for supplying fluid fuel to said gas producer chamber, and means for supplying a blast of air thereto, an exhaust conduit, a pipe for conducting air under pressure, means for connecting either of said flues with said pipe, and the other with said exhaust conduit, and means in said flues for condensing metallic vapors, and for separating from said flues the liquefied metal resulting from the condensation of said vapor.
8. In an apparatus of the character described, the combination of a furnace having a rear wall, through a central opening in which ore to be treated is charged, said rear wall being formed immediately beneath said charging opening with a small opening for 85 permitting the passage of a gas to said furnace through the body of ore charged thereto from said charging opening, and said apparatus having a gas producer chamber connected with said small opening, means for supplying fluid fuel to said gas producer chamber, and means for supplying a blast of air thereto, an exhaust conduit, a pipe for conducting air under pressure, means for connecting either of said flues with said pipe, and the other with said exhaust conduit, and means in said flues for condensing metallic vapors, and for separating from said flues the liquefied metal resulting from the condensation of said vapor.
9. In an apparatus of the character described, the combination of a furnace having a rear wall, through a central opening in which ore to be treated is charged, said rear wall being formed immediately beneath said charging opening with a small opening for 90 permitting the passage of a gas to said furnace through the body of ore charged thereto from said charging opening, and said apparatus having a gas producer chamber connected with said small opening, means for supplying fluid fuel to said gas producer chamber, and means for supplying a blast of air thereto, an exhaust conduit, a pipe for conducting air under pressure, means for connecting either of said flues with said pipe, and the other with said exhaust conduit, and means in said flues for condensing metallic vapors, and for separating from said flues the liquefied metal resulting from the condensation of said vapor.

In testimony whereof I have hereunto set my hand in the presence of two subscribing witnesses.

JOHN A. POTTER.

Witnesses:

W. W. BOUGHTON,  
JOEL T. TRAYLOR.